

## UNITED STATES PATENT OFFICE

2,177,160

## METHOD OF TREATING VENEERS

Frank V. Tischer, Dayton, Ohio; Anna M. Tischer, executrix of said Frank V. Tischer, deceased, assignor to Anna M. Tischer

No Drawing. Application November 23, 1936,  
Serial No. 112,308

3 Claims. (Cl. 21—23)

This invention relates to a method of treating veneers and to a composition for use in practicing that method.

When a veneer is subjected to moisture it swells in thickness and in width but does not swell appreciably in length. This is due to the fact that the length of the fibers of the wood is firmly established by nature while the spaces between the substantially parallel fibers are filled with hydroscopic matter which serves to unite the fibers into an integral structure. When a log is cut into veneers it must be cut in sections across the fibers of the wood to produce the desired configuration or "figure" in the veneer and as a result in many cases the veneer contains both straight or longitudinal grain and end or cross grain. In the ordinary process of veneering liquid glue is applied to the veneer and the latter is then applied to the core or body of the panel or other structure to which it is to be attached and the panel subjected to pressure in a press. The application of moisture to the veneer causes the straight grains to swell, thus increasing the thickness of the straight grain portions of the veneer while the end grain portions do not increase appreciably in thickness and this inequality cannot be corrected by the pressure to which the panel is subjected. As a result of this inequality in thickness of the different portions of the veneer air pockets are formed which prevent the proper adherence of the veneer to the core and result in the formation of blisters in the finished product.

One object of the invention is to provide a method of treating veneers to prevent the formation of blisters in the finished product.

A further object of the invention is to provide a method of so treating a veneer that the straight grain and end grain will be maintained at equal thickness and the straight grain will not swell when subjected to moisture.

A further object of the invention is to provide a method of treating a veneer to render the matter between the fibers thereof non-hydroscopic.

A further object of the invention is to provide a composition with which a veneer may be treated to produce the above mentioned results.

Other objects of the invention may appear as the method is described in detail.

In practicing the method I apply to the veneer, preferably to both sides thereof, a composition which will act on the matter between the wood fibers to render the same non-hydroscopic, then dry the veneer and subject the same to pressure and heat to cause the composition to penetrate

the veneer and to eliminate any inequality in the thickness of the straight grain and end grain.

The composition with which the veneer is treated comprises a suitable acid oxidizing agent which is dissolved in water and then reduced by a suitable alkali until it is neutral to litmus paper. A solution of about 10 Baumé in strength gives satisfactory results but, of course, the strength may vary.

Preferably in the preparation of the composition I dissolve two pounds of animal hide glue in one gallon of water, by the addition of heat, and add to the solution while hot one pint of a neutralized oxidizing agent in solution. The composition thus formed is then spread on the veneer, preferably on both sides thereof, and the coated veneer is then allowed to dry. The time required for proper drying varies, according to the character of the veneer, from one to twelve hours in a room temperature of 65 to 70° F. and about 40 to 50 relative humidity. The dry coated veneer is then placed between hot plates and subjected to pressure. Preferably the plates are steam heated and have about thirty to forty pounds steam pressure and about one hundred pounds per square inch weight pressure, and with such plates the pressure is continued for a period varying from one to five minutes, according to the requirements of the veneer. The action of the heat and pressure on the neutral oxidizing agent and the acid moisture of the veneer causes the composition to penetrate the veneer and to oxidize the glue and the hydroscopic matter between the wood fibers, thus rendering the latter nonhydroscopic. The pressure plates tend to equalize the thickness of all parts of the veneer and the latter, when removed from the press, is flat and of equal thickness in the straight grain and in the end grain thereof. The glue in the composition is not deteriorated by the action of the heat and the composition provides the veneer with a surface to which glue, subsequently applied thereto, will readily adhere. The pressure plates are preferably of iron as the coated veneers will not adhere to iron plates but may be readily removed therefrom.

When a veneer which has been so treated is subsequently attached to the core or body of the panel by the application of liquid glue thereto the straight grain will not swell, due, I believe, to the fact that the matter between the wood fibers has been oxidized and thus lost its ability to absorb moisture. As a result the panel, of which the veneer forms a part, is entirely free from blisters.

Any suitable oxidizing agent and alkali may

be employed in the forming of the composition but I prefer to use bichromate of potash or bichromate of soda as an oxidizing agent and to neutralize the same by the addition of sodium carbonate and sodium chloride. The three ingredients are employed in approximately equal quantities, say about one-half pound of each to a gallon of water. I prefer these ingredients because they are easy to combine, inexpensive and the solution so formed is stable throughout the year and, further, the dried coating formed by this composition adheres readily to glue subsequently applied. However, other ingredients may be used, such as nitric acid as an oxidizing agent and aluminum hydroxid or lead hydroxid as the neutralizing agent.

While the use of glue in the composition is desirable it is not essential to the oxidation of the hydroscopic matter and this may be accomplished without the use of glue.

While I have described the preferred method of practicing my invention and the preferred composition for use therein I wish it to be understood that I do not desire to be limited to the details thereof as various modifications may occur to one skilled in the art.

Having now fully described my invention, what I claim as new and desire to secure by Letters Patent, is:

1. A method of treating a veneer prior to gluing to render the hydroscopic matter therein non-hydroscopic, which comprises coating both sides of the veneer with a composition including a neutralized oxidizing agent and glue, drying the 5 coated veneer and subjecting the dried coated veneer individually to pressure in the presence of heat to cause said oxidizing agent to penetrate the veneer and act on the hydroscopic matter therein.

2. A method of treating a veneer prior to gluing to render the hydroscopic matter therein non-hydroscopic, which comprises coating both sides of the veneer with a composition including a neutralized oxidizing agent and glue, drying the 15 coated veneer and subjecting the dried coated veneer individually to pressure between hot metal plates to cause said oxidizing agent to penetrate the veneer and act on the hydroscopic matter therein and to flatten the surfaces of said veneer. 20

3. A method of treating a veneer prior to gluing to render the hydroscopic matter therein non-hydroscopic, which comprises coating both sides of a veneer with a solution including an acid oxidizing agent, an alkali and glue, drying the 25 coated veneer and subjecting the dried coated veneer individually to pressure between hot metal plates.

FRANK V. TISCHER.